

1

3,161,562

**PULPING CELLULOSE MATERIAL WITH AN ALKALINE COOKING LIQUOR CONTAINING HYDRAZINE**

Athey G. Gillaspie, Hamilton, Ohio, assignor to Champion Papers Inc., a corporation of Ohio  
No Drawing. Filed Dec. 13, 1960, Ser. No. 75,476  
9 Claims. (Cl. 162—72)

This invention relates to a method of producing cellulosic pulp such as wood pulp by the digestion of lignocellulosic materials with alkaline pulping liquors. In particular, it relates to the cooking of such materials in the presence of an agent which apparently inhibits the consumption of the alkaline reagents in those reactions in the pulping process which consume alkali without solubilizing lignin, thereby making the alkaline reagents more effective pulping materials.

In the conventional pulping processes a charge of lignocellulosic material, such as wood chips, straw, bamboo chips, or the like, is digested in a closed vessel at an elevated temperature in the range of about 300° to 370° F. and at corresponding pressures, usually in the range of 66 to 172 pounds per square inch. The alkaline process, as its name implies, is carried out at an alkaline pH. Sodium hydroxide may be the sole pulping agent present, as in the so-called "soda process." Mixtures of sodium hydroxide and sodium sulfide together with a certain amount of sodium carbonate are employed in the kraft or sulfate process. Between 30 and 90 grams per liter of these agents, calculated as Na<sub>2</sub>O, are normally employed; expressed another way, the amount of active reagent in the liquor is usually between 15% to 20% and most often between 16% and 18%, calculated as Na<sub>2</sub>O, on the dry weight of the lignocellulosic material, for the production of pulps which are to be bleached.

In the various alkaline pulping processes and modifications thereof, the combination of the high alkalinity and elevated temperatures and pressures employed in the digestion, have certain deleterious effects that are more or less accepted as necessary evils. Although the lignin is converted into removable form and the cellulose fibers are liberated, at the same time under these severe conditions, certain desirable materials such as the hemi-celluloses are dissolved and thereby lost, the lignin degradation products present in the wood and wood pulping medium are partially transformed into dark color-bodies which impair the color of the cellulose, and the cellulose chains are to some extent hydrolyzed or broken. As a result more material is removed than is necessary and the yield is low, in the range of 43% to 48% bleachable pulp on the weight of the wood used. If the cooking were less drastic, less of the hemi-cellulose would be removed and less of the smaller molecule carbohydrates would be split into the shorter chain lengths, and as a result, higher yields of pulp could be obtained. It should be possible in the case of fully cooked pulps to increase yields to 50% to 60% after pulping and still have a pulp of comparable strength and appearance. Retention of more of the hemi-cellulose would be advantageous as such material aids in the beating of the pulp and development of strength properties of the paper. Furthermore if the pulping could be modified to lessen or avoid the formation of color-bodies, the fibers should be easier to bleach. Moreover, if less severe conditions could be employed, a decided improvement in the strength of the pulp could be achieved; there would be less degradation of the cellulose, with better chain length as shown by higher disperse-viscosity values.

While it is known that mild cooking can be secured by reducing the caustic content, this ordinarily must be compensated by a substantially increased cooking cycle. In a

2

commercial operation it is not desirable for economic reasons to increase the cooking time unnecessarily.

An object of this invention is therefore an improved method of pulping cellulosic material such as wood pulp.

Another object of this invention is an improved process of pulping coniferous woods.

Still another object of this invention is a pulping process for lignocellulosic materials which requires a significantly reduced amount of alkali.

A further object of this invention is a pulping process for lignocellulosic materials which results in an increased yield of pulp.

An additional object of this invention is a method of producing a pulp of superior properties.

Other objects of this invention will be apparent from the disclosure herein.

In accordance with this invention it has been found that an addition of hydrazine to alkaline pulping liquors in certain proportions significantly increases the yield of delignified fibers and in addition produces a pulp of unusually high viscosity and improved brightness. By replacing a portion of the conventional pulping alkali reagents with hydrazine the less drastic cooking conditions result in less removal of the hemicellulose and less splitting of the smaller molecule carbohydrates.

While it is not completely understood why the use of hydrazine in an alkaline digestion liquor results in a greatly improved pulping process, it is believed to be due to the affinity of hydrazine for carbonyl groups in the cellulose. This affinity results in stabilization of the cellulose in such a manner as to make the caustic selective in its action against the lignin. Apparently the hydrazine causes the alkali to first react with the lignin and other readily removable materials, leaving the cellulose and hemicellulose intact. In this regard it has been established by experimentation with a fully bleached pulp that hydrazine does not prevent alkali from attacking cellulose; because of this it appears to subdue such action until all of the non-cellulosic or more readily reactive materials present in the chips are dissolved. While it is recognized that a number of reducing agents have been suggested in the literature as a means to facilitate pulping, none of these afford as significant a modification in regard to both yield and pulp properties as is obtained by the use of hydrazine. For this reason it appears that the action of hydrazine is an alkaline pulping system is not merely due to its reducing properties alone.

The hydrazine and alkali must be employed in certain proportions in the pulping liquor in order to obtain a beneficial digestion of the pulp. If hydrazine is employed in a full strength pulping liquor containing the usual 15 to 20% active alkali, calculated as Na<sub>2</sub>O, and based on the dry weight of the wood, the full shielding effect of the carbonyl groups by the hydrazine is not realized. For this reason the hydrazine is ordinarily effective only when no more than about 13% of active alkali calculated as Na<sub>2</sub>O, and based on the dry weight of the wood is used. It has been found that a maximum yield of a pulp of the most desirable properties is ordinarily obtained when the Na<sub>2</sub>O content does not exceed 10%. Since the wood chips are not defibered fully when less than 7% of alkali is employed it will usually be desirable to work within the particularly effective range of 7% to 10% alkali. If a semi-chemical pulping is desired it is possible to use 3% to 7% alkali followed by a mechanical defibering operation. The hydrazine will ordinarily be employed in the range of 12% to 30% based on the dry weight of the wood chips. Amounts in excess of 30% such as up to 40%, usually provide little or no additional benefit. Moreover, below 12% of hydrazine there is a gradual failure to completely shield the cellulose

from the caustic. Below 8%, the hydrazine has little or no effect.

The pulping liquor will contain water, the conventional alkali and other ingredients in addition to hydrazine and the wood chips. Sodium hydroxide, being readily available, is the preferred alkali although other alkali metal hydroxides such as potassium hydroxide may also be employed. Sodium sulfide and other sulfides will be present in the liquor used in the sulfate process. Inert ingredients which are ordinarily present in the cooking or "white liquor" used in the sulfate process are sodium carbonate, sodium sulfate, sodium sulfite, etc. The hydrazine hydrates can be used in place of hydrazine provided the amount of  $\text{NH}_2\text{NH}_2$  present for the reaction is within the amount specified.

The yield of pulp produced with the alkali hydrazine liquors in accordance with this invention is generally in the range of 50% to 56% and occasionally as high as 60%, based on the initial amount of wood chips, or about 10% to 15% higher than that obtained with a conventional kraft liquor. The increased yield of pulp and the need for using substantially less than the conventional amount of alkali results in a highly efficient process.

The method of this invention is particularly useful with coniferous woods, especially pines, since these present a much greater problem in pulping to obtain a high yield of a product of desirable properties. There is generally much less difficulty with the hardwoods in obtaining high yields having desirable P.N. values and correspondingly suitable viscosities.

Since the pines are normally pulped by the kraft or sulfate process using a mixture of sodium hydroxide and sodium sulfide, the hydrazine is particularly useful therewith. A further reason for the use of sodium sulfide is that it serves as a poison for ions that might otherwise catalyze the dangerous and explosive decomposition of hydrazine in an alkaline system.

The conditions of the pulping process, other than the reduced alkali content, are generally the same as employed in the conventional pulping operations. Ordinarily the presence of hydrazine permits the use of temperatures and pressures which are somewhat lower than the normal range of about 300 to 370° F. and 66 to 172 pounds per square inch. Even with hydrazine the use of temperatures and pressures much below the minimum of these ranges results in an incomplete removal of lignin. Where only a partial cooking is required, however, less drastic conditions can be employed. The ratio of the alkaline

considered a constituent of the liquor when expressing ratios of liquor to chips.

A further advantage of the process of this invention is improved quality of the pulp in regard to the amount of agent required to bleach it. In conventional digestion of wood chips, the cooking is carried to a point where the yield of pulp, basis dry wood before bleaching, is between 43-48%, and the permanganate number (P.N.) is between 16 and 20 for softwoods. The P.N. is an indication of the oxygen demand of the unbleached pulp (brown stock) which, in turn, is an indication of the amount of lignin and other reducing material left on the fibers that must be removed by the bleaching operation. In other words, the higher the P.N. number the greater amount of chlorine (and other bleaching agents) needed. The P.N. is not strictly quantitative but is merely an indication for any one pulping or bleaching system.

Pulps produced in accordance with this invention generally have P.N. values which are slightly lower than those produced by a conventional operation. Moreover, a pulp produced by this invention actually bleaches much more easily than a conventional kraft pulp which has a similar P.N.; i.e., a brightness of 80 can usually be obtained in four stages instead of the normal five or six stages. The hydrazine pulps are therefore characterized by ease of bleaching.

Still another important feature of the hydrazine pulping process is that the strength of the pulp is not materially lowered as it is in a conventional pulping operation. A measure of the strength of pulp is the Cupri-ethylenediamine Disperse Viscosity of Pulp, TAPPI standard T-230mm-50. This disperse viscosity is a measure of the chain length of the cellulose molecules present in the fibers, and is an indication of the amount of degradation due, initially, to the pulping operation, and later to the bleaching operations. The superior viscosity of the hydrazine pulp is reflected in better mullen and fold values before bleaching and partial development of these properties immediately upon bleaching.

Brightness values given herein were measured on a General Electric brightness meter.

The following examples will serve to further illustrate the invention.

#### Example I

A sample of mixed pine chips is pulped by the Kraft process (using sodium hydroxide and sodium sulfide as the active alkali) as follows:

| Sample       | Chips, Ovn dry Weight (Grams) | Active $\text{Na}_2\text{O}$ (percent by wt. based on chips) | Sulfidity (percent by wt. based on total alkali) | Activity | Liquor: Chips  | $\text{NH}_2\text{NH}_2$ Content (percent by wt. on dry wt. chips) | Yield of Pulp (percent based on O.D. chips) | P.N.         | Viscosity    | Brightness   |
|--------------|-------------------------------|--------------------------------------------------------------|--------------------------------------------------|----------|----------------|--------------------------------------------------------------------|---------------------------------------------|--------------|--------------|--------------|
| Control..... | 2,000<br>2,000                | 16<br>8                                                      | 28<br>28                                         | 88<br>88 | 3.7:1<br>3.7:1 | 0<br>30                                                            | 45.3<br>54.3                                | 15.7<br>14.3 | 17.8<br>38.3 | 26.4<br>38.0 |

hydrazine liquor to cellulosic material such as wood chips should be within the normal range of about 3:1 to 5:1. The sulfidity content of kraft pulping liquors should ordinarily not exceed 40% by weight based on the total alkali and most often should be in the range of 15% to 35%.

The standard terms used herein to designate chemicals in a cook are those defined by the Technical Association of the Pulp and Paper Industry. The total chemical in a cook is the weight of all sodium salts expressed as  $\text{Na}_2\text{O}$ . The total alkali is the weight of  $\text{NaOH} + \text{Na}_2\text{S} + \text{Na}_2\text{CO}_3 + \text{Na}_2\text{SO}_4$  all expressed as  $\text{Na}_2\text{O}$ . The active alkali is the weight of  $\text{NaOH} + \text{Na}_2\text{S}$  given as  $\text{Na}_2\text{O}$ . Activity equals the weight of active alkali divided by the weight of titratable alkali ( $\text{NaOH} + \text{Na}_2\text{CO}_3 + \text{Na}_2\text{S}$  all expressed as  $\text{Na}_2\text{O}$ ). The sulfidity is the weight of sulfide expressed as  $\text{Na}_2\text{O}$  divided by the weight total titratable alkali. As employed herein, the hydrazine is

The samples are pulped in a closed digester at 350° F. for 100 minutes after taking 60 minutes to attain this temperature. It is observed that the sample containing hydrazine generated slightly greater pressure than that containing no hydrazine.

It can be seen from this example that the use of hydrazine at reduced  $\text{Na}_2\text{O}$  content provides nearly a 10% increase in yield although pulping to substantially the same hardness, i.e., about 15. In addition the hydrazine pulp has a much greater brightness and viscosity than the control sample pulped in the absence of hydrazine.

The unbleached hydrazine pulp of Sample I actually requires a lesser period of ball milling or hydration in order to obtain a pulp having the most suitable mullen, tear and fold than does the Control or conventional pulp. At this shorter period of hydration the respective properties of the hydrazine pulp are equal to or superior to

those of the conventional pulp even at its extended hydration period. The ease of hydration of the hydrazine pulp is even further accentuated by bleaching.

Using on both Control and Samples I a conventional 6 stage bleaching sequence in the order of (percent of total chlorine, calculated as  $\text{Cl}_2$ ); (1) 53% chlorine, (2) 33% calcium hypochlorite, (3) sodium hydroxide extraction, (4) 10% calcium hypochloride, (5) sodium hydrox-

### Example III

This example illustrates the effect of variations of the hydrazine and chemical contents ( $\text{NaOH} + \text{Na}_2\text{S}$ ) of several cooks. All samples are cooked at a 4:1 liquor to chip ratio for a period of 60 minutes to attain 350° F. and then a period of 100 minutes at 350° F. The wood is again a chipped southern pine.

| Sample    | Active $\text{Na}_2\text{O}$ , percent by wt. based on chips | Sulfidity, percent by wt. based on total alkali | Activity, Percent | $\text{NH}_2\text{NH}_2$ content, percent by wt. on dry wt. chips | Final pH of Liquor | Yield Screened, percent on O.D. chips | Yield Total, percent based on O.D. chips | P.N.  | Viscosity | Remarks                                                                                                                                                                                                                                                                                      |
|-----------|--------------------------------------------------------------|-------------------------------------------------|-------------------|-------------------------------------------------------------------|--------------------|---------------------------------------|------------------------------------------|-------|-----------|----------------------------------------------------------------------------------------------------------------------------------------------------------------------------------------------------------------------------------------------------------------------------------------------|
| I-----    | 17                                                           | 25                                              | 88                | 0                                                                 | 11.3               | 45.8                                  | 45.9                                     | 16.6  | 23.3      | Normal pulping operation.                                                                                                                                                                                                                                                                    |
| II-----   | 3.4                                                          | 100                                             | -----             | 12.8                                                              | 9.8                | 58.2                                  | 70                                       | 126.0 | -----     | Use of all sulfide results in no pulping at this level.                                                                                                                                                                                                                                      |
| III-----  | 5                                                            | 25                                              | 88                | 19.2                                                              | 10.9               | 61.7                                  | 62.7                                     | 87.1  | -----     | Use of very low alkali content results in mere softening of chips and very little pulping. Essentially a semi-chemical pulp. The softened chips were defibered mechanically in a disc refiner by a single pass using stainless steel surfaces at a clearance of less than about 0.0001 inch. |
| IV-----   | 8                                                            | 25                                              | 88                | 19.2                                                              | 11.3               | 54.7                                  | 55.1                                     | 15.2  | 56.6      | Good results using hydrazine with reduced alkali content.                                                                                                                                                                                                                                    |
| V-----    | 8                                                            | 25                                              | 88                | 12.8                                                              | 10.7               | 46.8                                  | 53.8                                     | 30.5  | -----     | Inadequate pulping because of insufficient hydrazine at this alkali content. About 7% does not pass through screen.                                                                                                                                                                          |
| VI-----   | 10                                                           | 25                                              | 88                | 12.8                                                              | 11.0               | 46.7                                  | 50.0                                     | 15.7  | 65.2      | Good product although yield not as high as when greater amount of hydrazine used.                                                                                                                                                                                                            |
| VII*----- | 10                                                           | 25                                              | 88                | 19.2                                                              | 11.2               | 54.5                                  | 55.0                                     | 15.6  | 52.0      | Yield greatly increased with amount of hydrazine in spite of shorter cooking cycle.                                                                                                                                                                                                          |

\* This sample cooked at 350° F. for only 60 minutes.

ide extraction, and (6) 4% calcium hypochlorite the following results were obtained:

| Sample                | $\text{Cl}_2$ Applied, percent by wt. on Oven Dry Pulp | $\text{Cl}_2$ Consumed, percent by wt. on Oven Dry Pulp | Brightness   | Viscosity (centipoises) |
|-----------------------|--------------------------------------------------------|---------------------------------------------------------|--------------|-------------------------|
| Control Sample I----- | 8<br>7.4                                               | 7.35<br>6.4                                             | 78.9<br>85.4 | 8.0<br>15.3             |

From the above it will be seen that the bleached hydrazine pulp resulted in a much higher brightness and viscosity than the conventional pulp bleached by the same sequence.

### Example II

| Sample          | Chips, Oven Dry Weight | Active $\text{Na}_2\text{O}$ (percent by wt. based on chips) | Activity, Percent (approx.) | $\text{NH}_2\text{NH}_2$ Content (percent by wt. on dry wt. chips) | Pressure Raising Period, Min. To 350° F. | Full Pressure Period, Min. At 350° F. | Appearance of Pulp | Yield Total, percent by wt. based on chips | P.N.  | Viscosity |
|-----------------|------------------------|--------------------------------------------------------------|-----------------------------|--------------------------------------------------------------------|------------------------------------------|---------------------------------------|--------------------|--------------------------------------------|-------|-----------|
| Control A*----- | 50                     | 0                                                            | 0                           | 12.8                                                               | 40                                       | 100                                   | Bright-Unpulped    | -----                                      | ----- | -----     |
| Control B-----  | 2,000                  | 20                                                           | 100                         | 0                                                                  | 60                                       | 100                                   | Light Brown        | 24.8                                       | 29.5  | 11.3      |
| I*-----         | 50                     | 10                                                           | 100                         | 19.2                                                               | 45                                       | 100                                   | Light              | 52.6                                       | 18.8  | 21.6      |

\* As a safety factor, these were performed in a bomb reactor.

Control A shows that hydrazine in the absence of alkali does not facilitate pulping. Control B shows a normal soda pulping with a characteristic low viscosity and poor yield. In Sample I a pulp is obtained in an increased yield with an excellent P.N. and viscosity yet only half the normal amount of alkali has been employed. While the effect of hydrazine is not as significant in the absence of sulfide, nevertheless it is apparent that the efficiency of the pulping is increased by its presence.

Having thus disclosed the invention it will be apparent that various modifications thereof may be made which appear within the spirit of the invention and the scope of the claims.

I claim:

1. The method of producing a cellulosic pulp which comprises cooking a cellulosic material with an aqueous alkaline cooking liquor containing an amount of hydrazine which is at least about 8% by weight based on the dry weight of the cellulosic material.

2. The method of claim 1 wherein the aqueous alkaline cooking liquor contains no more than about 13% active alkali, calculated as  $\text{Na}_2\text{O}$  and based on the dry weight of the cellulosic material.

3. The method of claim 1 wherein the cellulosic material comprises wood chips.

4. The method of claim 3 wherein the wood chips are coniferous wood chips.

5. The method of producing wood pulp which comprises exposing wood chips to an alkaline cooking liquor at an elevated temperature and pressure, the said liquor containing about 7% to 13% active alkali, calculated as  $\text{Na}_2\text{O}$  and based on the dry weight of chips, and 8%

to 30% by weight of hydrazine, based on the dry weight of the chips.

6. The method according to claim 5 wherein the said liquor has a sulfidity content of 15% to 40%.

7. The method according to claim 5 wherein the said wood chips are coniferous wood chips.

8. Method according to claim 5 wherein the said liquor contains 7% to 10% active alkali, calculated as Na<sub>2</sub>O and based on the dry weight of the chips, and 12% to 30% hydrazine, based on the dry weight of the wood 10 chips.

9. The product produced by the method of claim 5.

References Cited in the file of this patent

UNITED STATES PATENTS

|           |                |       |               |
|-----------|----------------|-------|---------------|
| 2,071,304 | Hirschkind     | ----- | Feb. 16, 1937 |
| 2,909,446 | Redfarn et al. | ----- | Oct. 20, 1959 |
| 3,042,575 | Hartler        | ----- | July 3, 1962  |

FOREIGN PATENTS

|         |               |       |               |
|---------|---------------|-------|---------------|
| 846,079 | Great Britain | ----- | Aug. 24, 1960 |
|---------|---------------|-------|---------------|

UNITED STATES PATENT OFFICE  
CERTIFICATE OF CORRECTION

Patent No. 3,161,562

December 15, 1964

Athey G. Gillaspie

It is hereby certified that error appears in the above numbered patent requiring correction and that the said Letters Patent should read as corrected below.

Column 2, line 46, for "is an" read -- in an --; line 56, after "alkali" insert a comma; column 4, line 37, for "pulp" read -- pulps --; line 46, for "Kraft" read -- kraft --; columns 5 and 6, Example III chart, seventh column, in the heading after "percent" insert -- based --; same chart, last column, opposite Sample VII\*, after "with" insert -- greater -- same columns 5 and 6, Example II chart, column 9, line 2 thereof for "24.8" read -- 42.8 --;

Signed and sealed this 13th day of July 1965.

(SEAL)

Attest:

ERNEST W. SWIDER  
Attesting Officer

EDWARD J. BRENNER  
Commissioner of Patents